

Patented May 23, 1950

2,508,714

## UNITED STATES PATENT OFFICE

2,508,714

## PROCESS OF TREATING KERATINOUS MATERIALS

Milton Harris, Bethesda, Md., and Alfred E. Brown, Washington, D. C., assignors to Harris Research Laboratories, Washington, D. C., a partnership

No Drawing. Application October 7, 1946,  
Serial No. 701,623

8 Claims. (Cl. 8—102)

1

The present invention relates to the treatment of keratinous materials, such as wool, hair, fur and the like, and to the product of such treatment.

These materials are characterized by the presence therein of keratin, a fibrous protein containing amino acids including cystine. The amino acids are joined together by peptide linkages to form protein chains and the resulting chains are cross linked by the disulfide group (—S—S—) of cystine.

It is an object of the invention to provide an improved process for treating keratinous materials. A further object is to provide a process for stripping color from wool and like materials. Yet another object is to produce a modified keratinous material having improved chemical properties combined with substantially unimpaired physical properties.

One application of the invention is in the stripping of color from wool. In preparing wool products such as shoddy, clippings, rags and the like, for reprocessing, it is necessary to remove the dye or color from the wool. The present-day practice is to strip colors from wool in acidic media with sodium or zinc formaldehyde sulfoxylate. This treatment adversely affects the mechanical as well as the chemical properties of the wool even when the processing conditions are carefully controlled. Both the wet and dry tensile strength are decreased, especially the former, and often the wool acquires a dead and harsh "hand" as compared with the untreated material. This problem is accentuated with types of colors which are more difficult to strip and with which the concentration of the stripping agent or the duration of the treatment must be increased. In some cases a second strip is essential to remove the color and in these cases chemical damage to the wool is further increased. Wool products stripped by these conventional procedures also show an increased susceptibility to damage when treated under oxidizing, reducing or alkaline conditions in subsequent processing.

By the process of the present invention it is possible not only to strip color from wool without substantial impairment of the mechanical properties of the wool, but, quite apart from stripping, our process is useful in treating wool to improve its chemical properties and enhance its resistance to attack by oxidizing, reducing and alkaline agents.

In accordance with the invention, the keratinous material is subjected to the action of a re-

5

ducing agent for keratin in the presence of an alkylene dihalide.

The action of reducing agents on keratinous material ordinarily results in rupture of disulfide linkages and damage to the fiber. In our process, however, the linkages ruptured by the reducing agent are immediately rebuilt with the formation of new stable linkages. We provide an effective, commercially practical process for replacing relatively unstable chemical bonds of keratinous materials with new chemical linkages which are resistant to the action of oxidizing, reducing and alkaline agents.

The invention is illustrated by the following examples of procedures by which it may be put into practice:

## Example 1

1.5 parts of 1, 2-dichloroethane are dispersed in 450 parts of borate solution adjusted to pH 8.6. 7.5 parts of sodium sulfoxylate-formaldehyde are dissolved in the mixture, after which 15 parts of wool are immersed in the liquid. The temperature is raised to 80° C. and held for one hour, after which the wool is removed, rinsed and dried.

## Example 2

9.8 parts by weight of 1, 2-dibromoethane are dispersed in 3000 parts of 1% borax by means of a small amount of a quaternary salt of a substituted fatty acid amide available commercially under the trade name Sapamine KW. Any good dispersing agent may be used. 5 parts of sodium hydrosulfite are dissolved in the mixture, after which 100 parts of colored flannel rags are immersed in the liquor, and the mixture is kept at the boil for 15-30 minutes. The wool is then rinsed and dried. The color is stripped from the wool by this treatment.

## Example 3

1.5 parts of 1, 2-dibromoethane are dispersed in 450 parts of borate buffer, pH 8.6, after which 0.7 part of sodium hydrosulfite are added. 15 parts of old red knits are added. The mixture is treated at 80° C. for 30-60 minutes, after which the wool is rinsed and dried. The color is stripped from the wool by this treatment.

## Example 4

31.6 parts of 1,2-dibromoethane are dispersed in 4800 parts of water adjusted to pH 8.3 with borate solution. A convenient procedure is to use the required amount of a concentrated dispersion of 1,2-dibromoethane in water which can

be prepared with the aid of small amounts of sorbitan monostearate and the polyoxyalkylene derivative thereof, available commercially under the trade name Span 60 and Tween 60, respectively. 8 parts of sodium hydrosulfite are dissolved in the solution. 160 parts of black worsted shoddy are then immersed in the mixture and the entire reaction mixture is brought to the boil with occasional stirring. After one-half hour, the wool is removed, rinsed and dried. The color is stripped from the shoddy by this treatment.

*Example 5*

45 parts of 1,2-dibromoethane are dispersed in 11,500 parts of water and the pH adjusted to 15 8.5 with borate buffer, after which 45 parts of sodium hydrosulfite are added. 455 parts of wool cloth are added to this mixture. The entire mixture is then heated at 90-95° C. for one hour, after which the wool is rinsed and dried. The cloth is bleached lightly by this treatment. This treatment is also suitable for use with raw wool stock.

*Example 6*

1.5 parts of 1,2-dibromoethane are dispersed in 450 parts of borate buffer, pH 8.2, after which 0.7 part of formamidinesulfonic acid are added. 15 parts of blue serge rags are then added and the mixture is treated at the boil for 30-60 minutes, after which the wool is rinsed and dried. The color is stripped from the serge by this treatment.

*Example 7*

1.3 parts of 1,2-dibromoethane are dispersed in 420 parts of 0.3 molar borate solution, by means of cetyl dimethyl benzyl ammonium chloride available commercially under the trade name Triton K-60, and 0.7 part of sodium sulfoxylate-formaldehyde are then dissolved in the mixture. 15 parts of pastel sweater worsteds clippings are immersed in the mixture and the reaction carried out at the boil for 30 to 60 minutes, after which the wool is washed and dried. The color is stripped from the worsteds by this treatment.

In general, the alkylene dihalides employed as alkylating agents in the foregoing examples are not completely miscible in water. It is advantageous in practice first to form a concentrated dispersion of the alkylating agent in water by the use of small amounts of suitable dispersing agents such as those available commercially under the trade names of Sapamine KW, Triton K-60, Span 60, Tween 60, and other dispersing agents having a similar action. This concentrated dispersion is then added in appropriate amount to the solution containing the reducing agent, thus forming a suitable bath for the practice of our invention.

The process of the invention is subject to variation, for example in the reducing and alkylating agents used and the concentration thereof, the time of treatment, the temperature and pH of the bath, etc.

Examples of suitable reducing agents are the various sulfoxylate-formaldehyde compounds, the hydrosulfites, formamidine sulfonic acid and the like. Other reducing agents may be used, but they should be of a type which does not react with the alkylating agent (as would thiol compounds such, for example, as thioglycolic acid and salts thereof, monothioethylene glycol, and other mercaptans), since otherwise the two components of the solution would be exhausted by reaction with each other and would not be

available for reaction with the wool. The term "reducing agent" as used in the claims includes sulfoxylate formaldehyde compounds, hydrosulfites, formamidine sulfonic acid, and such other reducing agents for keratin as do not react with alkylene dihalides.

In the case of stripping processes, the choice of reducing agent will depend on the cost and the quality of the strip and will also depend upon the type of dye or color to be removed. Small scale trials will quickly indicate the best set of conditions to use for any given batch of goods. In some cases a much better strip can be obtained by first giving the wool an ammonia scour, for example with 2% to 5% of ammonia on the weight of the wool for thirty minutes at 50° to 60° C.

The amount of reducing agent employed may be varied over wide limits, up to 100% or more on the weight of the wool, with no appreciable effect on the properties of the modified wool produced. In stripping processes, in general 3 to 5% of the reducing agent on the weight of the wool will give an effective stripping action. Larger amounts may be present in the reaction mixture without significant adverse effect on the quality of the stripped product. With colors which are difficult to strip, it is advantageous to add the reducing agent in increments at the boil, since maximum reducing power for stripping purposes is thus utilized.

Suitable alkylating agents are the alkylene dihalides and substituted and modified alkylene dihalides, for example, methylene dibromide, 35 methylene diiodide, methylene bromoiodide, ethylene dibromide, ethylene dichloride, ethylene chlorobromide, trimethylene dibromide, 1,4-dibromobutane, 1,4-dichloro-2-butene, 2,2'-dichlorodiethyl ether, 4,4'-chloromethyl diphenyl and 40 2,2'-dibromo-diethyl ether. The term "alkylene dihalide" as used in the claims includes substituted and modified alkylene dihalides.

Very little alkylating agent is required; as little as 0.00045 mol of alkylating agent per gram of 45 wool gives good results. Larger amounts have no deleterious effect.

It has been found desirable to maintain the pH of the solution at 7 or above and preferably at pH 8-10. Adjustment of the pH to the value 50 desired can be made, for example, with alkaline salts such as borate or phosphate buffer or with borax.

The liquor-wool ratio may be varied over a wide range with no significant differences in the 55 proportion of the wool derivative formed. We prefer to employ liquor-wool ratios between about 10 to 1 and 40 to 1.

The process is operative and effective within a wide range of temperatures. We prefer to carry 60 out the treatment at temperatures between about 60° C. and 100° C.

The duration of the treating time may be varied considerably. After the desired amount of modification of the keratinous material has occurred, 65 further treatment will not significantly change the properties of the modified keratin product. In general, treatment for about one-half hour to one hour at 80° C. or from about one-quarter hour to one hour at the boil gives good results.

With the proper amount of alkylating agent present, the number of stabilized linkages that can be formed in the fiber will depend on the concentration of reducing agent, the pH of the solution and the temperature and duration of 70 the treatment. The keratinous products treated

in accordance with our invention exhibit significantly enhanced resistance to deterioration when exposed to oxidizing, reducing or alkaline agents. At the same time the mechanical properties of the wool are substantially unimpaired and are comparable to those of untreated wool.

It has been proposed to treat keratin with a reducing agent and subsequently to treat the resulting product with an alkylating agent. This treatment, however, results in a product essentially different from and markedly inferior to that obtained by our invention, when the same reducing agents are used. In the two-step process, deterioration of the fiber produced by the reducing agent persists in the final product to a substantial extent. The subsequent treatment with an alkylating agent is not capable of restoring to the keratin its original properties.

While our invention is not limited to any theory of operation, it is suggested that the alkylating agent in the reducing solution, by forming stable linkages immediately upon rupture of the disulfide linkages, preserves the physical properties of the material.

When keratinous material is treated with reducing agent alone, under the conditions of our treatment, a substantial number of sulfhydryl groups is formed, as indicated by a strong nitroprusside reaction. The mechanical properties of wool so treated are markedly inferior to those of the untreated product—its tensile strength is greatly weakened and the fabric becomes stiff and boardy. In our process, however, the detrimental effects noted with reducing agent alone are negligible.

Our process is capable of easy control. It is relatively insensitive to small variations in conditions such as temperature, concentration of reagents, time of treatment, etc. No damage is caused either by high concentrations of reducing agent or by unduly prolonged treatment.

We claim:

1. The process for modifying a keratinous material to increase its resistance to attack by oxidizing agents, reducing agents and alkalis while preserving substantially unimpaired its mechanical properties, which comprises treating the keratinous material at a temperature between 60° C. and 100° C. and a pH above 7, in a liquid bath containing 3% to 100% of the weight of the keratinous material of a reducing agent for keratin which is inert to alkylene dihalides, to rupture disulfide cross linkages of the keratinous material, said bath also containing more than 0.00045 mol per gram of keratinous material of an alkylene dihalide, whereby new stable alkylene cross linkages between the peptide chains of the keratin are formed immediately upon rupture of the disulfide linkages.

2. The method of stripping color from dyed wool while preserving substantially unimpaired the mechanical properties of the wool and increasing the resistance of the wool to attack by oxidizing agents, reducing agents and alkalis, which comprises treating the wool at a temperature between 60° C. and 100° C. and a pH above 7, in a liquid bath containing 3% to 100% of the weight of the wool of a reducing agent for keratin which is inert to alkylene dihalides and which is a stripping agent for dyestuff on wool, to rupture disulfide cross linkages of the wool and simultaneously strip the dyestuff, said bath also containing more than 0.00045 mol per gram of wool of an alkylene dihalide, whereby new stable alkylene cross linkages between the pep-

tide chains of the wool are formed immediately upon rupture of the disulfide linkages.

3. The method of removing color from wool while preserving substantially unimpaired the mechanical properties of the wool and increasing the resistance of the wool to attack by oxidizing agents, reducing agents and alkalis which comprises treating the wool at a temperature between 60° C. and 100° C. and a pH above 7, in a liquid bath containing 3% to 100% of the weight of the wool of a keratin reducing agent selected from the class consisting of sulfoxylate formaldehyde compounds, hydrosulfites and formamidine sulfonic acid, to rupture disulfide cross linkages of the wool and simultaneously remove color, said bath also containing more than 0.00045 mol per gram of wool of an alkylene dihalide, whereby new stable alkylene cross linkages between the peptide chains of the wool are formed immediately upon rupture of the disulfide linkages.

4. The method of stripping color from dyed wool while preserving substantially unimpaired the mechanical properties of the wool and increasing the resistance of the wool to attack by oxidizing agents, reducing agents and alkalis, which comprises treating the wool at a temperature between 60° C. and 100° C. and a pH above 7, in a liquid bath containing 3% to 100% of the weight of the wool of a keratin reducing agent which is a dyestuff stripping agent selected from the class consisting of sulfoxylate formaldehyde compounds, hydrosulfites and formamidine sulfonic acid, to rupture disulfide cross linkages of the wool and simultaneously strip the dyestuff, said bath also containing more than 0.00045 mol per gram of wool of 1,2-dibromoethane, whereby new stable alkylene cross linkages between the peptide chains of the wool are formed immediately upon rupture of the disulfide linkages.

5. The method of stripping color from dyed wool while preserving substantially unimpaired the mechanical properties of the wool and increasing the resistance of the wool to attack by oxidizing agents, reducing agents and alkalis, which comprises scouring the wool with 2% to 5% of its weight of ammonia at a temperature between 50° C. and 60° C. and then treating the wool for from  $\frac{1}{4}$  hour to 1 hour at a temperature between 60° and 100° C. and a pH above 7, in a liquid bath containing 3% to 100% of the weight of the wool of a reducing agent selected from the class consisting of sulfoxylate formaldehyde compounds, hydrosulfites and formamidine sulfonic acid, to rupture disulfide cross linkages of the wool and simultaneously strip the dyestuff, said bath also containing more than 0.00045 mol per gram of wool of an alkylene dihalide, whereby new stable alkylene cross linkages between the peptide chains of the wool are formed immediately upon rupture of the disulfide linkages.

6. The method of removing color from wool while preserving substantially unimpaired the mechanical properties of the wool and increasing the resistance of the wool to attack by oxidizing agents, reducing agents and alkalis which comprises treating the wool at a temperature between 60° C. and 100° C. and a pH above 7, in a liquid bath containing 3% to 100% of the weight of the wool of sodium sulfoxylate formaldehyde, to rupture disulfide cross linkages of the wool and simultaneously remove color, said bath also containing more than 0.00045 mol per gram of wool of an alkylene dihalide, whereby new stable alkylene cross linkages between the pep-

peptide chains of the wool are formed immediately upon rupture of the disulfide linkages.

7. The method of removing color from wool while preserving substantially unimpaired the mechanical properties of the wool and increasing the resistance of the wool to attack by oxidizing agents, reducing agents and alkalis, which comprises treating the wool at a temperature between 60° C. and 100° C. and a pH above 7, in a liquid bath containing 3% to 100% of the weight of the wool of sodium hydrosulfite, to rupture disulfide cross linkages of the wool and simultaneously remove color, said bath also containing more than 0.00045 mol per gram of wool of an alkylene dihalide, whereby new stable alkylene cross linkages between the peptide chains of the wool are formed immediately upon rupture of the disulfide linkages. 10

8. The method of removing color from wool while preserving substantially unimpaired the mechanical properties of the wool and increasing the resistance of the wool to attack by oxidizing agents, reducing agents and alkalis, which comprises treating the wool at a temperature between 60° C. and 100° C. and a pH above 7, in a liquid bath containing 3% to 100% of the weight of the 20

wool of formamidine sulfonic acid, to rupture disulfide cross linkages of the wool and simultaneously remove color, said bath also containing more than 0.00045 mol per gram of wool of an alkylene dihalide, whereby new stable alkylene cross linkages between the peptide chains of the wool are formed immediately upon rupture of the disulfide linkages. 15

MILTON HARRIS.

ALFRED E. BROWN.

#### REFERENCES CITED

The following references are of record in the file of this patent:

#### UNITED STATES PATENTS

| Number    | Name          | Date          |
|-----------|---------------|---------------|
| 2,019,124 | Evans         | Oct. 29, 1935 |
| 2,180,262 | Sturm         | Nov. 14, 1939 |
| 2,206,535 | Lubs          | July 2, 1940  |
| 2,261,094 | Speakman      | Oct. 28, 1941 |
| 2,297,701 | Hugh          | Oct. 6, 1942  |
| 2,403,906 | Burke         | July 16, 1946 |
| 2,403,937 | Lubs          | July 16, 1946 |
| 2,418,071 | Harris et al. | Mar. 25, 1947 |
| 2,434,562 | Harris        | Jan. 13, 1948 |